

Oct. 8, 1963

D. R. EASTMAN ET AL.  
PHOTOCONDUCTOGRAPHY EMPLOYING ELECTROLYTIC  
IMAGES TO HARDEN OR SOFTEN FILMS  
Filed July 28, 1960

3,106,516



Fig. 1



Fig. 2



Fig. 4



DONALD R. EASTMAN  
RAYMOND F. REITHEL  
INVENTORS

BY *R. Frank Smith*  
*Emerson Holmes*  
ATTORNEYS

# United States Patent Office

3,106,516

Patented Oct. 8, 1963

1

3,106,516

## PHOTOCONDUCTOGRAPHY EMPLOYING ELECTROLYTIC IMAGES TO HARDEN OR SOFTEN FILMS

Donald R. Eastman and Raymond F. Reithel, Rochester, N.Y., assignors to Eastman Kodak Company, Rochester, N.Y., a corporation of New Jersey

Filed July 28, 1960, Ser. No. 45,950

10 Claims. (Cl. 204—18)

This invention relates to photoconductography.

Photoconductography forms a complete image at one time or at least a non-uniform part of an image as distinguished from facsimile which at any one time produces only a uniform dot. The present invention would be useful with facsimile but finds its greatest utility in photoconductography.

Cross reference is made to the following series of co-filed applications:

Serial No. 45,940, John W. Castle, Jr., "Photoconductography Employing Reducing Agents."

Serial No. 45,941, Raymond F. Reithel, "Photoconductolithography Employing Nickel Salts," continuation-in-part Serial No. 120,863, filed June 7, 1961.

Serial No. 45,942, Raymond F. Reithel, "Photoconductolithography Employing Magnesium Salts."

Serial No. 45,943, Raymond F. Reithel, "Photoconductography Employing Spongy Hydroxide Images," continuation-in-part Serial No. 120,035, filed June 27, 1961.

Serial No. 45,944, Raymond F. Reithel, "Method for Making Transfer Prints Using a Photoconductographic Process."

Serial No. 45,945, Raymond F. Reithel, "Photoconductography Employing Manganese Compounds."

Serial No. 45,946, Raymond F. Reithel, "Photoconductography Employing Molybdenum or Ferrous Oxide," continuation-in-part Serial No. 120,036, filed June 27, 1961.

Serial No. 45,947, Raymond F. Reithel, "Photoconductography Employing Cobaltous or Nickelous Hydroxide," continuation-in-part Serial No. 120,037, filed June 27, 1961.

Serial No. 45,948, Donald R. Eastman, "Electrophotolithography."

Serial No. 45,949, Donald R. Eastman, "Photoconductolithography Employing Hydrophobic Images."

Serial No. 45,951, Donald R. Eastman and Raymond F. Reithel, "Photoconductography Employing Absorbed Metal Ions," continuation-in-part Serial No. 120,038, filed June 27, 1961.

Serial No. 45,952, Donald R. Eastman and Raymond F. Reithel, "Photoconductography Employing Spongy Images Containing Gelatin Hardeners."

Serial No. 45,953, John J. Sagura, "Photoconductography Employing Alkaline Dye Formation," now Patent No. 3,057,787.

Serial No. 45,954, John J. Sagura, and James A. Van Allan, "Photoconductography Employing Quaternary Salts."

Serial No. 45,955, Franz Urbach and Nelson R. Nail, "Uniform Photoconductographic Recording on Flexible Sheets."

Serial No. 45,956, Franz Urbach and Nelson R. Nail, "High Contrast Photoconductographic Recording."

Serial No. 45,957, Nicholas L. Weeks, "Photoconductography Involving Transfer of Gelatin."

Serial No. 45,958, Donald R. Eastman, "Photoconductolithography Employing Rubeanates."

Serial No. 45,959, Donald R. Eastman and Raymond F. Reithel, "Electrolytic Recording with Organic Polymers."

2

Serial No. 46,034, Franz Urbach and Donald Pearlman, "Electrolytic Recording."

Electrolytic facsimile systems are well known. Electrolytic photoconductography is also known and is described in detail in British 188,030, Von Bronk, and British 464,112, Goldman, modifications being described in British 789,309, Berchtold, and Belgian 561,403, Johnson et al.

The present invention is closely related to our cofiled application Serial No. 45,952 listed above entitled "Photoconductography Employing Spongy Images Containing Gelatin Hardeners."

Since it involves hardening or softening of gelatin and/or organic polymers it is also related to the cofiled applications listed above by Eastman and Reithel entitled 15 "Electrolytic Recording With Organic Polymers," and by Urbach and Pearlman entitled "Electrolytic Recording." It differs from the cofiled application Serial No. 45,953 listed above of Sagura having to do with "Alkaline Dye Formation" in that it relates to hardening 20 and softening of separate sheet materials.

The present invention in certain embodiments involves the direct deposition of gelatin on a photoconductor.

In the present invention the photoconductographic image is used to control the solubility of gelatin or of 25 certain polymers coated on a separate sheet. The object of the invention in this connection is to provide a process which yields prints of better contrast than are obtained when the final image is formed directly on the photoconductive layer by electrolytic deposition from an 30 electrolyte useful in photoconductography. Also the recording layer itself carrying the gelatin or polymer need not be electrically conducting.

Other objects of the invention depend on how the hardened or softened layer is utilized. The object of the 35 invention thus is to provide a photoconductographic process which produces any one of the following results:

- A. Single copy
- B. Lithographic master
- C. Spirit master
- D. Stencil master
- E. Colloid transfer master (bearing an operational similarity to that described in U.S. Patent 2,596,756)
- F. Dye imbibition master
- G. Magnetic printing master
- H. Ion transfer master

The invention can also be used for making negative or positive transparencies.

The following known phenomena are utilized in the 50 practice of this invention:

Gelatin hardening: The processes of tanning or hardening of gelatin by certain organic or inorganic chemicals are well-known reactions and are the bases of many important photocopying and photochemical processes. Es- 55 pecially, some gelatin hardening agents, e.g. cobalt salts or co-polystyrene maleamic acid are effective only above a certain pH value. Dry layers coated from acid STAM-gel solutions are relatively insoluble in aqueous media above this critical pH value. STAM is the ammonium salt of styrene maleamic acid copolymer and STAM and gelatin dissolved in water constitutes a STAM-gel solution.

Gelatin softening (solubilization): It is also well 60 known that aqueous solutions of certain inorganic chemicals, e.g. potassium alum ( $K_2Al_2(SO_4)_4 \cdot 24H_2O$ ) are effective hardening agents of lime-processed gelatin only within a narrow pH range (pH between 3–6). Within this range, the melting point of gel layers, so hardened, is much higher than at lower or higher pH values. Raising the pH softens gelatin which has been so hardened. Unhardened lime-processed gelatin layers also show a

marked dependence of melting point on pH but the differential is not nearly as pronounced as with potassium alum hardened gels.

Synthetic polymer solubilization: Dry layers of certain synthetic organic polymers of the general class represented by cellulose acetate phthalate, polymethyl methacrylate comethacrylic acid, or STAM are insoluble in acidic aqueous solutions, but can be rendered soluble in alkaline media.

Synthetic polymer insolubilization: Layers of other organic polymers of the class represented by polyvinyl pyridine are soluble in aqueous acid media but insoluble in alkaline media. Coated from acid solutions, these layers can be insolubilized by contact with alkaline solutions.

The visibility or lack of visibility of the electro-deposited material (i.e. the "image") on the photoconductive surface is irrelevant to the practice of this invention.

This invention is essentially a two-step process in which the first step is electrolytic and the second chemical. With various subsequent treatments, such as wash-off, this second chemical step produces (1) a physical change, (2) a differential in mechanical or thermo-mechanical properties, (3) a differential in dye absorbtivity, and/or (4) a differential in receptivity to "greasy" lithographic inks, when wetted with the proper press fountain solutions.

Specifically, this invention consists of the imagewise electrolytic deposition, on a photoconductive surface, of a material (an image) which, by itself or by chemical reaction with other agents in the recording layer, will harden or soften gelatin or insolubilize or solubilize polymers.

The invention will be fully understood from the examples given below and from the following description when read in connection with the following drawings in which:

FIG. 1 is a schematic flow chart illustrating a preferred embodiment of the invention.

FIG. 2 similarly illustrates an alternative to one step of the process shown in FIG. 1.

FIGS. 3, 4 and 5 illustrate various printing processes utilizing the gelatin relief which results from the present invention as shown in FIG. 1.

In FIG. 1 a transparency 10 is illuminated by a lamp 11 and an image thereof is focused by a lens 12 on a photoconductive zinc oxide in resin layer 15 carried on a conducting support 16. The transparency is moved to the left as indicated by the arrow 17 and the photoconductor, as indicated by the arrow 18, moves synchronously with the image of the transparency 10.

While the photoconductivity image persists in the zinc oxide layer 15, it is passed under a brush 20 containing an electrolyte. A potential difference is maintained between the brush 20 and the roller 21 by a source of potential indicated schematically at 22. The zinc oxide layer is the cathode as shown, but A.C. potential may be applied since the zinc oxide in contact with the electrolyte acts as a rectifier so that it is a cathode in the electrolytic action. The electrolyte contains magnesium ions and an image 23 of magnesium hydroxide is deposited on the exposed areas of the photoconductor 15. Then according to the invention, this image is pressed into contact with a gelatin or polymer layer 30 carried on a suitable support 31, pressure being applied by rollers 32. The layer 30 is such that it is hardened or softened when raised to the pH of magnesium hydroxide. In the case where it is hardened, or insolubilized, a supply of water 37 washes off the relatively soft or soluble areas and leaves a relief image 35 on the support 31.

Alternatively, as shown in FIG. 2, when the layer 30 is a hard one, softened by the magnesium hydroxide image 23, the spray of water 37 washes off the areas thus softened and leaves a relief image 38 on the support 31. Either of these relief images resulting from FIG. 1 or FIG. 2 may be used in any of the subsequent reproduc-

tion processes. For simplicity, the relief image 35 is the one illustrated in FIGS. 3, 4 and 5.

In FIG. 3 the relief image is used for imbibition printing. An imbibition dye 41 is applied by a roller 40 to the relief image 35, for example an image of gelatin. This relief image is then pressed into a receiving sheet 43 and the dye transfers as indicated at 44. This FIG. 3 could also illustrate the use of the relief image as a spirit transfer master. In this case the dye is applied to the relief or is included in the original gelatin layer and in the presence of alcohol a small portion of dye transfers to the receiving sheet. Similarly FIG. 3 could represent the application of magnetic material to the relief for subsequent use in magnetic printing.

The sheet 31 may be either hydrophilic or hydrophobic and the image 35 may be hydrophobic or hydrophilic. In the arrangement shown the support 31 is a hydrophobic sheet and the image 35 is a gelatin which is hydrophilic even when hardened with formaldehyde. In FIG. 4, 10 this layer of gelatin is moistened by a roller 50 which applies a standard fountain solution 51. The plate is then inked with a standard litho greasy ink 53 by a roller 52, the ink adhering as shown at 54 to the areas of the support 31 which are not covered by the image 35. In the 15 usual offset method this ink is transferred to an offset drum 57 as indicated at 58 and is printed on a succession of sheets of paper such as shown at 59.

An alternative lithoprinting system which has proven most satisfactory utilizes the standard litho materials 20 (e.g. Duplimat) supplied with office type litho presses, particularly for use with colloid transfer processes. These standard sheets will receive and hold soft gelatin which, in such colloid transfer processes for making litho plates, is hardened and rendered hydrophobic. The sheet is then 25 treated with a solution which renders the support hydrophilic, for standard lithoprinting on an office litho printer such as supplied by the Addressograph-Multigraph Corporation.

In the present invention this Duplimat material is utilized with differentially hardened gelatin as shown schematically in FIG. 5. The differentially hardened gelatin layer with hardened areas 34 (corresponding to the relief areas 38 of FIG. 2) and with unhardened areas 33 is pressed in contact with a hydrophobic litho (Duplimat) master 61, pressure being applied by rollers 69. Part of the unhardened gelatin 33 transfers as shown at 63 to the support 61. This image is treated by swabbing with a brush 64 which applies a gelatin hardener, tannic acid, to harden the transfer image 63. The hardening in this 30 case is sufficient to make the gelatin hydrophobic. The whole sheet is then treated with a solution in a brush 65 which is the standard solution ("Platex") supplied with the sheet 61 to render the surface 62 thereof hydrophilic but leaving the hardened gelatin layer 63 hydrophobic. The 35 support 61 with the hydrophilic areas 62 and the hydrophobic areas 63 is now ready for lithoprinting on a standard press, the operation being schematically shown in FIG. 5. The moistening roller 50 applies a fountain solution 51 which wets the area 62. The inking roller 60 50 then applies a greasy ink to the image areas 63, the ink adhering to these areas as indicated at 70. Then in the usual way, the ink 70 transfers to an offset drum 71 as indicated at 72 and prints onto a sheet of paper 73 passed in contact with the drum 71.

The gelatin relief made in accordance with the present invention may be transferred to a silk screen to act as a stencil, for silk screen printing.

Examples of uses of solubility images are as follows:

Gelatin hardening: Since organic hardening agents such as formaldehyde, or p-quinone do not form useful electrolytic deposits (in cathodic operation) on ZnO photoconductive surfaces, it is necessary either (1) to apply these hardening agents to an absorbent imagewise deposit or (2) to co-deposit the hardening agent with a hydrous oxide forming material. The hardening rate and

efficiency of these organic agents increases with increased alkalinity. This alkalinity can be supplied in either or both of two ways, (1) by the alkalinity of the image deposit and/or (2) by adjusting the pH of the gelatin before coating.

Most of the inorganic hardening agents, e.g. potassium alum, chrome alum, cerium salts, etc. which do form hydrous electrolytic deposits from aqueous solutions of their soluble salts do not require the inclusion of other hydroxide-forming metal salts in the electrolytic developer. However, the deposition of the hydroxide of iron, for example, is improved by the inclusion of magnesium or manganese salts in the developer.

When the hardening agent, (e.g. co-polystyrene maleamic acid, or cobalt salts) is ineffective in acid media, the dry layers coated from acid gel solutions containing these agents can be insolubilized by contact with alkaline reactive electrolytic deposits, e.g.  $Mg(OH)_2$ .

Any pigments, dyes or other materials used in the process must not detrimentally soften or harden the gelatin or polymer or adversely affect its other properties.

The following ten systems represent preferred uses of hardened gelatin relief images:

(1) Single copy wash-off: An imagewise distribution of deposited hardening agent or hydroxy ions from an alkaline deposit it transferred by pressure contact, into a pigmented or dyed gelatin layer coated on a separate support. The unhardened gelatin is removed by washing in hot water. The resultant print is a positive if the exposure was made to a negative original. With certain gelatin layers, parts of the soft gelatin adheres to the zinc oxide layer in the non-image-bearing areas to produce a direct positive image on the zinc oxide surface; this is a useful added feature.

(2) Single copy thermo-mechanical transfer: An imagewise distribution of hardening agent, or hydroxyl ion from an alkaline deposit, is transferred, by pressure contact, into a pigmented or dyed gelatin layer on a separate substrate. The unhardened gel is then transferred by thermo-mechanical means onto a separate receiving sheet. If the photoconductor is exposed to a positive original, the remaining unhardened gel on the separate recording layer will be a negative copy, and the transferred gel on the receiving sheet a positive copy.

(3) Lithographic printing recording layer as master (wash-off): Gelatin hardened with formaldehyde repels "greasy" lithographic inks. With the gel recording layer on an ink-receptive substrate, a positive-to-positive lithographic printing master can be produced.

(4) Transfer to "Duplimat": The unhardened gelatin is transferred, by pressure contact, onto the surface of a gelatin-receptive "Multilith Type" sheet and the gelatin image rendered ink-receptive by chemical treatment (discussed in connection with FIG. 5 above). This provides a direct positive system.

(5) Spirit duplicating: If spirit soluble dyes are incorporated in the separate recording layer, the masters or prints obtained by method 1 or 2 will provide a suitable duplicating master for this system.

(6) Stencil duplicating: A gelatin impregnated silk screen or tea-bag paper (or any suitable open-mesh material) is contacted with a hardening-agent image-deposit. The unhardened gel areas are then removed by a wash-off step. This provides a direct-positive system.

(7) Colloid transfer master: The unhardened dyed and/or pigmented gelatin is transferred from the separate recording layer, by pressure-contact onto a series of suitable receiving sheets. A few copies can be obtained from a single master. This provides a positive-to-positive system.

(8) Dye imbibition printing: The gelatin image obtained either after wash-off or by transfer to a separate receiving sheet, will absorb dyes. As is common in dye transfer processes, these dyes can be transferred onto a separate receiving sheet.

(9) Magnetic printing: Magnetic printing masters, negative-to-positive or positive-to-positive depending on which of the above processes is used in making the relief, can be produced by incorporating magnetically hard materials in the recording layer.

(10) Ion transfer printing: Color-forming agents incorporated in the gelatin can be transferred, by use of a suitable solvent, into another layer containing other agents and upon chemical reaction form a visible image.

Gelatin softening (solubilization): For example, gelatin layers hardened with potassium alum can be solubilized, by contacting them with an alkaline image deposit, by virtue of the strong dependency of hardening efficiency upon pH. Such embodiments are particularly useful in the following two examples:

(1) Single copy wash-off: Wash-off of the softened (solubilized) areas provides a direct-positive copying system.

(2) Single copy transfer of softened gelatin: Transfer of the softened gel to a separate receiving sheet will provide a negative-to-positive process.

Polymer solubilization: The dry layers of these alkaline soluble polymers, coated from organic solvent solution, can be solubilized by contact with alkaline reacting image deposits. Even better results are obtained in this process if hydrophilic (wettable) pigments are used in the layer. This aids in obtaining the maximum degree of image-material transfer and penetration. Examples, particularly which have proven suitable to this embodiment of the invention, are as follows (four examples):

(1) Single copy: Hydroxyl ions from an alkaline image deposit are transferred, by pressure contact, into the dyed, or pigmented layer. The solubilized areas are then removed by wash-off. This furnishes a direct-positive copying process.

(2) Lithographic printing: When wetted with lithographic "wet-out" solutions, the areas contacted by the alkaline image deposit will repel "greasy" lithographic inks. The remaining areas are ink-receptive. This provides a direct-positive copying process.

(3) Stencil duplicating: A silk screen or tea-bag impregnated with one of these polymers is contacted with an alkaline image deposit, and the solubilized areas washed out. This provides a negative-to-positive copying process.

(4) Magnetic printing: Incorporation of hard magnetic materials in the polymer layers will provide a positive-to-positive system for producing a magnetic printing master.

The following specific examples of the various embodiments of the invention were all carried out with photoconductive layers which consisted of dye sensitized zinc oxide dispersed in a resin binder coated on an aluminum foil-paper-laminate support using electrolytic development which utilizes the persistency of photoconductivity exhibited by these layers. The invention can, of course, also be carried out in photoconductive processes involving simultaneous exposure and development. In all of the examples, the electrolysis was carried out with aluminum foil backing of the photoconductive layer held at a negative potential with respect to the counter electrode and the electrolytic developer was carried in a viscous sponge brush-type counter electrode.

#### Example 1

A gelatin recording layer was prepared as follows:

65 6 g. Grasol Fast Black "G" (Geigy dyestuffs)  
100 cc. of 2% gelatin lime-processed  
6 cc. ethyl alcohol

Ball mill for 18 hours in a pint-sized mill with 12 Borundum balls. Filter through a balloon silk filter bag. To 50 cc. of the above mixture was added:

70 50 cc. of 10% gelatin  
0.4 g.  $KNO_3$   
75 1.5 cc. glycerol

Filter through a balloon silk filter bag and coat 0.005 inch thick on electron bombarded titanox pigmented polyethylene treated paper stock.

Magnesium-formaldehyde: As one example of this invention, a dye-sensitized zinc oxide layer was exposed for 5 seconds to 500 ft. candle tungsten illumination through a 0.3 density increment photographic step-wedge. The resulting conducting image was developed electrolytically using a 1% magnesium nitrate hexahydrate plus 4% formaldehyde solution contained in a viscose sponge brush electrode, held at 70 volts, positive with respect to the zinc oxide layer with ten strokes development. The excess electrolyte was removed from the zinc oxide surface with an absorbent tissue. A sheet of the above prepared gelatin coating 0.005 inch wet thickness was moistened with cold tap water and rolled into contact with the zinc oxide layer containing the magnesium hydroxide-formaldehyde hardening image. After allowing 50 seconds for transfer of formaldehyde and hardening to occur, the gelatin layer was peeled from the zinc oxide surface and the soft gelatin was removed by a hot water rinse (140° F.). A hardened gelatin plus dye pigment relief image remained on the polyethylene coated sheet. A step-wedge image of soft gelatin remained on the zinc oxide layer in a pattern corresponding to areas of low exposure. The hardened gelatin step-wedge image indicated that an exposure of 125 ft.-candle-second was required on the zinc oxide layer to produce hardening of the gelatin from a photoconductive image produced as above. This example is also given in our coiled application on spongy images containing gelatin hardeners but is included here because it is not known whether the formaldehyde also deposits electrolytically.

#### Example 2

Chrome alum: As another example of this phase of the invention, a dye-sensitized zinc oxide layer was exposed for 5 seconds to 400 ft. candle tungsten illumination through a high-contrast line negative reversed from left to right. The conducting image was developed electrolytically using a 1% solution of chrome alum (potassium chromium sulfate tetracosahydrate) contained in a viscose sponge brush electrode, held at 70 volts potential positive with respect to the zinc oxide layer, and ten strokes development. The excess developer was removed from the zinc oxide layer using an absorbent tissue. A sheet of the gelatin layer prepared in Example 1 was moistened with cold tap water and rolled into contact, gelatin face to zinc oxide layer surface. After allowing 50 seconds for chrome alum transfer, the gelatin layer was peeled from the zinc oxide layer and the soft gelatin was removed by rinsing in 110° F. tap water for 10 seconds. A gelatin plugs pigment positive relief image of the negative was left on the polyethylene coated paper support.

For examples 3 and 4 gelatin layers were prepared in the following manner:

6.0 g. Grasol Fast Black "G"  
100 cc. 2% gelatin  
2 cc. ethyl alcohol

Ball mill for 67 hours in a pint-sized mill using 12 Borundum balls and add:

80 cc. 10% gelatin  
20 cc. distilled water

Filter through a balloon silk filter bag and coat at pH=6.5, pH=4.9 and pH=4.0 on titanox pigmented polyethylene coated paper stock BE7385C, 0.003 inch and 0.005 inch wet thickness.

#### Example 3.—Magnesium-Cerium

A sheet of dye-sensitized zinc oxide was exposed for 3 seconds to 400 ft.-candle tungsten illumination through a high contrast, line copy, negative transparency and developed as in Example 2 using a solution of 0.5% magne-

sium nitrate hexahydrate plus 1% cerous nitrate hexahydrate. Transfer was effected as in Example 2 using the gelatin layer 0.005 inch wet thickness with pH=6.5. After peeling the layers apart, 3 minutes were allowed for hardening before the soft gelatin was removed by 110° F. tap water.

#### Example 4.—Manganese-Iron

A sheet of dye-sensitized zinc oxide was exposed and developed as in Example 3 using a solution of 0.75% ferrous sulfate heptahydrate plus 0.5% manganous nitrate. Transfer was effected as in Example 3 using the gelatin layer coated 0.005 inch wet thickness with pH=4.0. After peeling the layers apart, 2 minutes were allowed for additional hardening before the soft gelatin was removed by rinsing in 120° F. tap water. Since it is possible that the iron as well as the hydrated oxide of manganese is being deposited electrolytically this constitutes an example of the present invention but if the iron is merely absorbed by the spongy hydrated manganese oxide image, it is an example of our coiled case.

#### Example 5—Cobalt

As another example of this invention, a gelatin layer was prepared in the following manner:

50 cc. 1% gelatin  
1.0 g.  $\text{Co}(\text{NO}_3)_2 \cdot 6\text{H}_2\text{O}$   
1 cc. glycerol  
2 cc. wetting agent

It was filtered through a balloon silk filter bag and coated 0.003 of an inch on polyethylene coated paper stock.

A sheet of dye-sensitized zinc oxide was exposed and developed as in Example 3 using a solution of 1% magnesium nitrate hexahydrate. A sheet of the above gelatin coating containing a cobalt salt was moistened with cold tap water and was rolled into contact with the above prepared magnesium hydroxide image. Hydroxyl ions transferred to the gelatin sheet and produced the hardening of gelatin by alkaline cobalt in 60 seconds transfer and hardening time. The layers were separated by peeling and the soft gelatin was removed by rinsing in 120° F. tap water for 10 seconds.

#### Example 6—STAM

A 5% STAM solution was made up as follows: Two lbs. of STAM (the ammonium salt of styrene maleamic acid copolymer) was stirred in 12 liters of distilled water containing 135 cc. of a 3%  $\text{NH}_4\text{OH}$  solution. Stirring was continued for 2 hours and the solution was kept overnight at room temperature, after which the final, net weight was adjusted to 18,160 g. with distilled water.

A dyed, alkali-hardenable STAM-gelatin layer was made up as follows:

To 200 g. of a 10% de-ashed gelatin at 40° C. containing 6 cc. of 7.5% saponin, 32 cc. of the 5% STAM solution was added with stirring. Within 30 seconds of the STAM solution addition, a mixture of 6 cc. of 28% acetic acid and 6 cc. of distilled water was added slowly.

The entire mixture was then stirred for 20 minutes at 40° C., set by chilling and stored under 40° refrigeration. A portion of the STAM-gelatin described above was then remelted at 40° C. and a water-soluble dye was added.

The dyed gel was then hand-coated on a titanox pigmented, polyethylene coated paper support with a 0.005 inch aperture doctor blade, was set by chilling and was air dried at room temperature, 50% R.H. for several days before use.

A piece of photoconductive, dye-sensitized zinc oxide was exposed for 0.5 second to 200 ft. candle tungsten radiation incident upon a high-contrast negative transparency in contact with the photoconductive surface, then brush developed at 60 volts with a viscose sponge wetted with an aqueous solution of 1% magnesium sulfate hepta-

hydrate (pH adjusted to 9.6 with 2% sodium hydroxide solution). The print surface was then dried by blotting with an absorbent tissue.

The surface of a sheet of the dyed STAM gel recording layer was moistened with distilled water, then was rolled into contact with the image-bearing zinc oxide surface. After 60 seconds, the recording layer was peeled off and the unhardened gel areas, corresponding to the areas of no image deposit, were washed off with 110° F. water.

Exposing the zinc oxide layer to a negative original resulted in a positive print on the recording layer.

*Example 7.—Lithographic Printing-Recording Layer as Master*

A gelatin layer was prepared as follows:

10 g.  $\text{Fe}_3\text{O}_4$   
100 cc. 2% gelatin  
2 cc. ethyl alcohol

Ball mill for 42 hours in a pint-sized mill with 12 Borundum balls. Add 100 cc. 10% gelatin. Filter through a balloon silk filter bag and coat 0.005 inch thick on polyethylene coated paper stock.

A dye-sensitized zinc oxide layer was exposed for 3 seconds to 400 ft. candle tungsten illumination through a positive line transparency and developed electrolytically as in Example 1. (Again this may be an example of hardening by the image or by the material in a spongy image depending on whether the formaldehyde is considered part of the image or merely in the image.) A sheet of the above gelatin coated paper was moistened and rolled into contact with the electrolytically produced magnesium hydroxide-formaldehyde image material. After allowing 50 seconds for formaldehyde transfer and hardening to occur, the sheets were separated by peeling. The soft gelatin was rinsed out of the image areas with 120° F. tap water revealing the hydrophobic polyethylene sheet. The wetted formalin hardened gelatin in the background was ink repellent. The sheet was forced air dried and mounted on a Multilith, Duplimat master and treated with Repelex fountain solution 1:32 dilution and run on a Multilith No. 500 press using Van Son Black No. 40904 ink. One hundred copies were made from the master.

*Example 8.—Spirit Master*

A gelatin plus spirit-soluble-dye recording layer was prepared as follows:

50 cc. of 5% gelatin  
0.1 g. methyl violet  
0.05 g. saponin

It was filtered through a balloon silk filter bag and coated 0.005 and 0.010 inch thick on polyethylene coated paper stock. A sheet of dye-sensitized zinc oxide was exposed for 3 seconds to 400 ft. candle tungsten illumination through a high-contrast line negative. The image was developed electrolytically as in Example 1. The image is a magnesium hydroxide formaldehyde material or is a spongy magnesium hydroxide with absorbed formaldehyde. A sheet of the above recording layer was moistened with tap water and rolled into contact with the zinc oxide layer containing the hardening image. Fifty seconds was allowed for transfer and hardening to occur. The gelatin layer was peeled from the zinc oxide surface and the soft gelatin was removed by a 3-second rinse in 130° F. tap water, and then was dried. A sheet of "Ditto" brand receiving paper was moistened with alcohol-NaOH mixture and rolled into contact with the gelatin plus dye image prepared above. Five seconds were allowed for transfer of dye and the receiving paper was removed. This was repeated with a second sheet etc. Ten copies were made to illustrate the multiple copy process.

*Example 9.—Verifax-Type Transfer Printing-Mechanical Transfer*

A gelatin transfer matrix was prepared as follows:

5 12. g. Grasol Fast Black "G"  
100 cc. 2% gelatin  
4 cc. ethyl alcohol

Ball mill for 5 hours in a pint-sized mill with 12 Borundum balls and filter through a balloon silk filter bag.  
10 Add 100 cc. of 20% gelatin. Filter again and coat 0.010 inch thick on polyethylene coated paper stock.

A dye-sensitized zinc oxide layer was exposed for 3 seconds to 400 ft. candle tungsten illumination through a positive transparency line copy. The conducting image 15 was developed electrolytically using a solution of 1% magnesium nitrate hexahydrate plus 4% formaldehyde at pH=8.5 with sodium hydroxide as in Example 1. A sheet of the above prepared gelatin layer was moistened with cold tap water and rolled into contact with the 20 above prepared image material. After allowing 50 seconds for formaldehyde transfer and hardening of the gelatin, the layers were separated by peeling and parts of the soft gelatin were transferred to Verifax copy paper by pressure rollers and peeling. Ten copies were made 25 from this one master.

*Example 10.—Thermo-Mechanical Stripping*

A gelatin transfer matrix was prepared as follows:

30 15 g.  $\text{Fe}_3\text{O}_4$  (ferromagnetic)  
100 cc. 2% gelatin

Ball mill for 52 hours in pint-sized mill with Borundum balls. Add:

35 1 g. Uni-Aga dispersed in 80 cc. distilled water at 75 C.  
20 cc. 10% gelatin  
2 cc. wetting agent

Filter through a balloon silk filter bag and coat 0.003 inch thick on polyethylene coated paper support.

40 A sheet of dye-sensitized zinc oxide was exposed (as in Example 9) for 1½ seconds. The layer was developed electrolytically as in Example 9. A sheet of the above-prepared gelatin coating was moistened and rolled into contact with the magnesium hydroxide-formaldehyde 45 image material. After allowing 50 seconds for formaldehyde transfer and hardening to occur, the sheets were separated by peeling. The gelatin coated polyethylene sheet containing the image hardened gelatin was run through heated rollers at approximately 120° F. in contact with a sheet of Verifax copy paper. The sheets were 50 separated by peeling and there was complete transfer of the soft gelatin to the Verifax copy paper to produce a positive reproduction, the hardened gelatin remaining on the polyethylene coated sheet in the form of a negative 55 reproduction. If exposure is made through a negative transparency, the useful positive image remains on the polyethylene coated sheet and the soft "background" gelatin transfers to the Verifax receiving sheet to produce a negative.

60 *Example 11.—Magnetic Printing Master*

A gelatin plus ferromagnetic pigmented recording layer was prepared in the following manner:

50 cc. of 2% gelatin (lime processed cattle-hide)  
65 3.0 g.  $\text{Fe}_3\text{O}_4$  (ferromagnetic)  
2 cc. ethyl alcohol

These compounds were mixed together in a pint-sized ball mill with 12 Borundum balls and milled for 18 hours. To the above mixture was added:

70 50 cc. of 10% gelatin  
0.4 g.  $\text{KNO}_3$   
0.5 g. Uni-Aga (from gelled concentrate) at 50° C.  
It was filtered through a balloon silk filter bag and coated 75 0.005 inch thick on polyethylene coated stock.

The process for producing a relief image here was the same as for Example 1 except that the exposure was made through a high-contrast line negative. The image (consisting of hardened gelatin plus  $\text{Fe}_2\text{O}_3$ ) was air dried and was magnetized by running one pole face of a bar magnet across the surface of the image material several times. The print was then bathed in a suspension of carbonyl iron in cyclohexane for 10 seconds. The print was allowed to dry and the carbonyl iron particles held by the magnetic image were transferred between pressure rollers to a specially treated pressure transfer paper. A carbonyl iron positive image resulted.

*Example 12.—Gelatin Softening-Single Copy-Wash Off*

A sheet of the Grasol Fast Black "G" pigmented recording layer (pH=4.9) described in Examples 3 and 4, was bathed for 60 seconds with agitation in 100 cc. of a 3%, by weight, potassium alum ( $\text{K}_2\text{Al}_2(\text{SO}_4)_4 \cdot 24\text{H}_2\text{O}$ —photographic grade) solution, was rinsed briefly with distilled water, then was air dried at room temperature for 20 hours before use. This prehardened gel layer was found to be insoluble in 104° F. water.

A piece of the photoconductive, dye-sensitized zinc oxide material was exposed for 1 second to 500 ft. candle tungsten radiation incident upon a high-contrast positive transparency in contact with the photoconductive surface and then was developed, electrolytically, at 60 volts with a viscose sponge wetted with an aqueous solution containing 1% by weight, magnesium nitrate hexahydrate the pH of which was adjusted to 9.5 with a 2% sodium hydroxide solution.

After electrolytic development, the print surface was dried by blotting with an absorbent tissue which removed the excess electrolyte from the non-image-bearing areas.

The gel surface of the recording layer was then moistened with cold water and was rolled into contact with the image-bearing photoconductive surface.

After 60 seconds, the recording layer was peeled off and the solubilized (softened) areas, corresponding to the areas of alkaline image-deposit, were removed by washing in running 104° F. tap water. The gel corresponding to the areas without image deposit was unaffected by this treatment. Exposure of the zinc oxide to a positive original produced a positive print on the recording layer.

*Example 13.—Single Copy: Polymer Solubilization*

5 g. of  $\gamma\text{-Fe}_2\text{O}_3$  was added to 100 ml. of ethyl alcohol in which was dissolved 5 g. of methylmethacrylate methacrylic acid (MMAX). The mixture was roll milled for 24 hours in a pint-size ceramic jar containing 12 Borundum balls, then was coated on titanox-pigmented, polyethylene-coated paper stock with a 0.003 in. aperture doctor blade and the layer air dried at room temperature for two days before use.

A piece of the photoconductive layer was exposed for 10 seconds to 400 ft. candle tungsten radiation incident upon a positive transparency in contact with the photoconductive surface, and then was electrolytically developed at 70 volts with an aqueous solution of 1% by weight, magnesium nitrate hexahydrate. The surface was then dried with an absorbent tissue.

The surface of a sheet of the  $\gamma\text{-Fe}_2\text{O}_3$  MAX layer was wetted with water and then was rolled into contact with the image-bearing photoconductive surface. The areas solubilized by contact with the alkaline magnesium hydroxide image material were then removed by washing with 140° F. tap water. During the washing, a cotton pad was rubbed on the surface to aid in removing the solubilized areas.

*Example 14.—Lithographic Master*

A solution consisting of 5% by weight of methylmethacrylate methacrylic acid dissolved in ethyl alcohol was used to coat a 0.005 in. (wet) layer on a Mylar (polyethylene terephthalate) support. The layer was then air dried at room temperature for several hours before use.

5 A piece of the dye-sensitized zinc oxide material was exposed for 5 seconds to 400 ft. candle tungsten radiation incident upon a high-contrast positive transparency in contact with the photoconductive surface and then was electrolytically developed at 70 volts with an aqueous solution containing 1% by weight, magnesium sulfate heptahydrate. The surface was then dried by blotting with an absorbent tissue.

10 The MAX layer surface was then wetted with distilled water and was rolled into contact with the image-bearing photoconductive layer surface.

15 After 60 seconds the layer was peeled off and its surface was wetted with a 1:7 dilution of Repelex fountain solution. The surface was then hand-inked with Kwik-lith Process Black No. 244388 carried on a plastic roller.

20 The areas of the MAX layer which had contacted the image-bearing areas of the photoconductive surface were ink-repellent. The remaining areas were ink-receptive.

*Example 15.—Silk Screen*

25 A piece of silk screen was impregnated with a 3% by weight MAX ethyl alcohol solution. The silk screen was dipped into the solution, then allowed to air dry at room temperature for several days before use.

30 A sheet of the photoconductive layer was exposed for 10 seconds to 400 ft. candle tungsten radiation incident upon a high-contrast negative transparency in contact with the photoconductive surface and then was electrolytically developed at 70 volts with an aqueous solution containing 1% by weight magnesium sulfate heptahydrate. The surface was then dried with an absorbent tissue.

35 The MAX impregnated silk screen was wetted with water, then was rolled into contact with the image-bearing photoconductive surface.

40 After 120 seconds, the silk screen was removed, and the areas solubilized by contact with the alkaline, magnesium hydroxide image deposit were washed out with hot water. The remaining areas were unaffected by this treatment.

The water-treated screen was then dried in forced air at room temperature.

45 An ink print was made by hand squeegeeing ink through the stencil onto a sheet of ink-absorbent paper.

*Example 16.—Magnetic Printing Master*

The print obtained in Example 13 was used as a magnetic printing master.

50 The  $\gamma\text{-Fe}_2\text{O}_3$  MAX image on the print was magnetized by drawing the print across one pole of a bar magnet.

55 The print was then dipped into a carbonyl iron-Freon 113 slurry. The carbonyl iron adhered to the image-material but not to the background.

The carbonyl iron was then pressure-contact transferred to a receiving sheet by passing between two steel rollers.

60 *Example 17.—Polymer Insolubilization*

A polymer layer was prepared as follows: 5 g. poly-2-vinyl-pyridine was added to 35 cc. distilled  $\text{H}_2\text{O}$  containing 2 cc. 12 N HCl.

65 The mixture was allowed to stand for a period of 14 hours. The undissolved material was filtered out and the following was added:

70 15 cc. 20% gelatin  
0.5 g. 5,5' indigo disulfonic acid disodium salt  
2 cc. wetting agent

The material was filtered through a balloon silk filter bag and coated 0.003 inch on titanox pigmented polyethylene coated paper stock.

75 The gelatin merely acts as a binder and other binders may be used. The treatment (discussed below) with

## 13

$Mg(OH)_2$  acts to soften the gelatin slightly; the main effect is the hardening and insolubilization of the polymer.

A sheet of dye sensitized zinc oxide coating on an aluminum foil paper laminate was exposed for 3 seconds to 400 ft. candle tungsten illumination through a high contrast line-copy negative transparency. The resulting conducting image was developed electrolytically, using a solution of 1% magnesium nitrate hexahydrate (pH = 9.0 with NaOH), held in a viscose sponge brush electrode, 70 volts positive with respect to the zinc oxide layer. The excess developer was removed from the photoconductor's surface with an absorbent tissue and the surface containing the basic magnesium hydroxide image wetted with a thin layer of distilled water. A sheet of the dry coating made as above was rolled into contact with the above prepared image material. After allowing 50 seconds for hydroxyl ion transfer and polymer insolubilization to occur the recording layer was peeled off and washed under warm water. The areas rendered insoluble by the  $Mg(OH)_2$  were unaffected by this wash treatment, whereas the areas corresponding to the non-image areas were dissolved off the recording layer leaving a relief image of dyed polyvinyl pyridine.

Example 18.—*Electrolytic Deposit of Gelatin*

In some of the coiled applications (e.g., Urbach and Nail, "Uniform Photoconductographic Recording on Flexible Sheets") gelatin was included in the electrolyte. A small amount of such gelatin aids in the deposit of metal or other image, but not enough gelatin comes down to be useful as a relief image. The present example, however, concerns the deposit of large amounts of gelatin, sufficient to be visibly dyed. We have found that gelatin containing cobalt ions or STAM-gelatin containing magnesium ions deposits electrolytically and forms a relief image directly.

It is noted that neutral or slightly acid, aqueous solutions of cobalt salts, e.g.,  $Co(NO_3)_2$ , are not effective as gelatin hardeners. However, in an alkaline medium (such as at the pH at which  $Co(OH)_2$  forms) cobalt becomes an effective hardening agent. This is utilized in the present example.

A sheet of dye sensitized zinc oxide in resin was exposed for 1 second to 500 foot candle tungsten radiation incident upon a high contrast line copy negative transparency in contact with the photoconductor. The imagewise conductivity pattern was then developed electrolytically with an aqueous electrolyte made up of 40 cc. of a solution of 5% lime processed gelatin (pH adjusted to 8.5 with 2% NaOH) and 10 cc. of a solution of 10% cobaltous nitrate hexahydrate.

A viscose sponge carrying the above developer electrolyte, held at 60 volt positive potential with respect to the aluminum foil backing of the photoconductor, was twice drawn slowly across the exposed surface. The surface was then rinsed with water at room temperature to remove any gel solution from the non-image-bearing areas. The image-bearing areas retained a relatively heavy gelatin relief image. The sheet was then air dried at room temperature.

For comparison with this gelatin image, another sheet of the same photoconductor was similarly exposed and, in this case, developed in an aqueous solution of 1% cobaltous nitrate hexahydrate (but with no gelatin). It was rinsed and air dried.

One-half of each print was dipped for several seconds into an aqueous solution of the dye 5,5'-indigo disulfonic acid disodium salt and rinsed under cold tap water. The image material on the gelatin developed layer absorbed the dye whereas the image developed without gelatin did not absorb dye.

## 14

## Example 19

This example is similar to Example 18 but using magnesium ions which at high pH harden STAM gelatin. The operation is the same. The electrolyte contained both magnesium nitrate and STAM gelatin. The STAM gelatin was found to deposit with the magnesium hydroxide and to form a STAM gelatin relief image which dyed readily.

Having described various examples of our invention, it is pointed out that it is not limited thereto but is of the scope of the appended claims.

We claim:

1. In a photocoductographic process in which an image pattern of variations in electrical conductivity is produced in a photoconductive layer, the steps of electrolytically cathodically depositing an alkaline image of magnesium hydroxide and placing said image directly in contact with an organic polymer layer whose solubility in water changes in the presence of alkaline magnesium hydroxide.
2. The process according to claim 1 in which the layer is gelatin which is hard at a pH lower than that of magnesium hydroxide and which is softened by said image.
3. The process according to claim 1 in which said layer is gelatin containing a hardening agent which is effective only above a pH value between neutral and that of magnesium hydroxide said agent being selected from the group consisting of cobalt salts and co-polystyrene maleamic acid, which layer is hardened by said image.
4. The process according to claim 1 in which said layer is a synthetic organic polymer selected from the group consisting of cellulose acetate phthalate and poly methyl methacrylate co-methacrylic acid which polymers are relatively insoluble in aqueous solutions with pH below 7 and which increase in solubility at the higher pH of magnesium hydroxide.
5. The process according to claim 1 in which said layer is primarily polyvinyl pyridine coated from an acid aqueous solution which layer is rendered substantially insoluble at the pH of magnesium hydroxide.
6. The process according to claim 1 in which the layer is gelatin which is differentially hardened by the image and the soft areas of which adhere to the photoconductor to form a gelatin relief.
7. In a photocoductographic process in which an image pattern of variations in electrical conductivity is produced in a photoconductive layer, the steps of electrolytically cathodically depositing chromic hydroxide distributed in accordance with said pattern from an electrolyte containing chrome alum and placing said deposited chromic hydroxide directly in contact with a gelatin layer which hardens in the presence of chrome alum.
8. Gelatin hardened by the addition of cobaltous ions at a pH greater than that at which cobalt hydroxide forms.
9. In a photocoductographic process in which an image pattern of variations in electrical conductivity is produced in a photoconductive layer, the steps of electrolytically cathodically depositing in accordance with said pattern an image containing a gelatin hardener selected from the group consisting of magnesium hydroxide and chrome alum and placing said deposited image directly in contact with a gelatin layer which hardens in the presence of said hardener.
10. A process according to claim 9 in which the gelatin layer contains a cobaltous salt.

## References Cited in the file of this patent

## UNITED STATES PATENTS

- 571,531 Langhans ----- Nov. 17, 1896  
 70 2,763,553 Clark et al. ----- Sept. 18, 1956

## FOREIGN PATENTS

- 215,754 Australia ----- June 23, 1958